

## [54] MEANS FOR DETERMINING THE OXYGEN CONTENT OF LIQUID METALS

[76] Inventor: George R. Fitterer, 825 Twelfth St. Oakmont, Pa., 15139

[22] Filed: Apr. 30, 1971

[21] Appl. No.: 138,985

## Related U.S. Application Data

[63] Continuation-in-part of Ser. No. 786,866, Dec. 23, 1968, Pat. No. 3,619,381, which is a continuation-in-part of Ser. No. 570,855, Aug. 8, 1966, abandoned.

[52] U.S. Cl. .... 204/195 S, 204/1 T

[51] Int. Cl. .... G01n 27/46

[58] Field of Search .... 136/86 F, 153; 204/1 T, 195 S

## [56] References Cited

## UNITED STATES PATENTS

|           |         |                    |           |
|-----------|---------|--------------------|-----------|
| 3,309,233 | 3/1967  | McPheeeters et al. | 204/195 S |
| 3,347,767 | 10/1967 | Hickam             | 204/195 S |
| 3,400,054 | 9/1968  | Ruka et al.        | 204/1 T   |
| 3,403,090 | 9/1968  | Tajiri et al.      | 204/195 S |
| 3,404,036 | 10/1968 | Kummer et al.      | 136/153   |
| 3,410,780 | 11/1968 | Holden             | 204/195 S |
| 3,442,773 | 5/1969  | Wilson             | 204/1 T   |
| 3,464,008 | 8/1969  | Meysson et al.     | 204/195 S |
| 3,468,780 | 9/1969  | Fischer            | 204/195 S |
| 3,471,390 | 10/1969 | Kibby et al.       | 204/195 R |
| 3,616,407 | 10/1971 | Engell et al.      | 204/195 S |

## FOREIGN PATENTS OR APPLICATIONS

21,673 8/1961 Germany .... 204/195 S

## OTHER PUBLICATIONS

Horsley "AERE Report R 3427," United Kingdom

Atomic Energy Authority, 1961, pp. 1-6 &amp; FIG. 2.

Turkdogen et al. "Rapid Oxygen Determination in Liquid Steel," 76th General Meeting of AISI, May 23, 1968, pp. 1-23.

Fitterer, "Reprint from Journal of Metals," Aug. 1966, pp. 1-6.

Primary Examiner—T. Tung

Attorney—Joseph M. Lane, Donald R. Dunner, Warren B. Kice, Richard L. Aitken and Robert F. Ziems

[57]

## ABSTRACT

A probe capable of being plunged into a high temperature liquid metal without destructive thermal shock for determining the dissolved oxygen content of the liquid metal comprises an elongated electrically insulating refractory envelope and a small mass of refractory oxide-type oxygen-anion permeable solid electrolyte material supported adjacent one end of the envelope. At least a portion of at least one side of the mass is exposed through an opening in the envelope for contact with the liquid metal, and the aforementioned side portion is disposed adjacent the one envelope end. Reference means are provided in the envelope for contacting an apposed side of the mass with an oxygen reference material. The probe is provided with circuit means extending into the envelope for electrically contacting the apposed side of the mass, together with additional circuit means disposed for electrically contacting the liquid metal for measuring an emf developed across the mass in proportion to the aforesaid dissolved oxygen content.

19 Claims, 13 Drawing Figures



Fig. 1.



Fig. 3.



Fig. 2.



Fig. 4.



Fig. 5.



Fig. 6.



Fig. 10.



Fig. 11.





Fig. 7.



Fig. 8.



Fig. 12.



Fig. 13.



Fig. 9.

## MEANS FOR DETERMINING THE OXYGEN CONTENT OF LIQUID METALS

This application is a continuation-in-part of my co-pending application entitled DETERMINING OXYGEN CONTENT OF MATERIAL, Ser. No. 786,866 filed Dec. 23, 1968, now U.S. Pat. No. 3,619,381, which in turn is a continuation-in-part of my then co-pending application Serial Number 570,855 filed Aug. 8, 1966, now abandoned.

The present invention relates to methods and means for the direct determination of oxygen content of various materials, and more particularly to means and methods for the substantially instantaneous determination of oxygen in liquid metals and other materials maintained at elevated temperatures, for example, molten steel. Certain arrangements of the invention are adapted for use with conductive and non-conductive materials, respectively, particularly at elevated temperatures.

There are many applications throughout industry wherein it is necessary to ascertain the oxygen content of various materials. However, in order for such information to be useful in many manufacturing processes, it is essential that the oxygen analyses be timely made to permit corrective adjustment of manufacturing processes. In the case of liquid steels and other high-temperature liquid metals, various methods have long been used for the sampling and analysis of their oxygen contents. In the manufacture of rimming steel, certain high quality steels, and other metals which are melted at high temperatures, it is essential that the quantity of oxygen or other gas dissolved in the steel be closely controlled. In various liquid metal processes, a technique for continuously monitoring the dissolved oxygen content is sorely needed, particularly for those high temperature liquid metals maintained at 800° C or 1,000° C and higher. In all of the analytical methods developed previously, however, it has been necessary to extract a sample of the molten steel or other liquid metal or alloy from the ladle or from the furnace as the case may be. The sample then is carried elsewhere for analysis, for example, by vacuum fusion procedures.

The analysis made in the foregoing manner is time-consuming, in addition to involving considerable labor costs, and does not provide an up-to-the-minute picture or analysis of gas content in the molten material during the manufacturing process. Therefore, corrective measures have to be delayed until the analysis becomes available from the laboratory. In consequence, such corrective measures usually are ineffective or at best serve merely to provide background or post-mortem information relative to succeeding heats, batches, or melts.

These difficulties are overcome by my disclosed direct-determination apparatus and methods which involve the insertion of a probe into a high temperature material such as molten steel or other liquid metal. In the case of liquid steels or the like, means are afforded for penetrating any overlying slag without affecting the reading. Upon contact with the liquid metal or other material, the probe through suitable electric circuitry yields an indication of the oxygen content substantially at the instant of insertion. In one arrangement of my apparatus, liquid metal or other high temperature material can be brought into contact with a solid electrolytic cell of specialized construction, when the probe is inserted therein. Such contact is established in a man-

ner so as to expose the electrolytic cell to the material having an unknown oxygen content, without either oxidation or deoxidation of the sample by contact with extraneous materials. The resultant electromotive force generated by the cell when contacted with the material is found to vary in direct proportion to the dissolved or uncombined oxygen content of the molten metal. A suitable calibration can be readily established to relate oxygen content to the *emf* value, depending upon temperature and the characteristic oxygen pressure developed by the reference material inside the probe. The *emf* is a function of the ratio of the oxygen pressure of the oxygen dissolved in the metal and the oxygen pressure exhibited by the reference material at the temperature of insertion.

In either case, the substantially instantaneous analysis of the oxygen content in the molten metal or other material at elevated temperatures is completed in a few seconds after the probe is inserted. Thus, useful manufacturing information can be obtained even where the oxygen level is changing rapidly. On the other hand, with previous analytical techniques, the values of oxygen content, even if accurate, would be useless insofar as that particular batch or heat would be concerned.

Most importantly, my apparatus is capable of being plunged into molten steel or other materials maintained at extremely high temperatures without fracturing or otherwise suffering destructive thermal shock. A measurement of the dissolved oxygen content is obtained, owing to the novel construction of my apparatus, at a predetermined point or location within the bath of molten steel or the like. Previous apparatus for this purpose have been subject to fracturing or other thermal shock when plunged into molten steel. Prior oxygen measuring devices used closed-end elongated tubes which were entirely composed of a stabilized, solid, oxygen-conducting electrolyte which in this form is not resistant to thermal shock.

The structural and technical disadvantages of the prior art which have been noted during the preceding discussion are illustrated by the U. S. Pats. to Hickam No. 3,347,767; Alcock No. 3,297,551; McPheeters et al No. 3,309,233; Kolodney et al No. 3,378,478; and Fischer No. 3,359,188. Each of these patents contemplates the provision of an elongated tube made from a solid electrolyte material. This representative sampling of the prior art emphasizes the inability of prior devices to measure the dissolved oxygen content of liquid metals without exceptionally slow preheating. That the relatively large electrolyte tube is subject to thermal shock is abundantly illustrated by Kolodney et al who provided a surrounding mesh basket for collecting pieces of the electrolyte tube upon fragmentation. These references further represent the difficulty of suitably insulating the walls of the electrolyte tube from its holder to prevent shorts in the electric circuit.

My apparatus, on the other hand, employs a probe using a relatively small mass of solid electrolyte, supported near the end of an elongated, insulating tube. The assembly thus formed is highly resistant to thermal shock, and only a very small area of the electrolyte is exposed to the high temperature material being measured. A further advantage arises from confining the measurement to a very small, predetermined point or area within the heat or melt.

A number of laboratory instruments for the direct measurement of oxygen have also been proposed from

time to time. These are typified by Horsley, AERA Report R3427 pp. 1-6 and FIG. 2, 1961. An electrolyte disc is sandwiched between two cermet electrodes for the purpose of measuring the free energy in the cermets. The sandwich is held together by a pair of tubes, an additional purpose of each of which is to supply a controlled, inert atmosphere respectively to the outward surfaces of the cermets. Further, the cermet discs are separated from the supporting tubes by nickel discs or foils. If the lower supporting tube of the Horsley device were removed, the entire assembly would, of course, fall apart. Obviously, there is no teaching of submerging the Horsley device in a liquid material particularly in a high temperature liquid material. Similarly, there is no teaching of securing a small mass or pellet of solid electrolyte material near the end of a supporting and insulating tube.

Similar apparatus for the direct measurement of oxygen is described in the literature, representative references to which are tabulated below:

1. K. Kiukkola and C. Wagner: J. Electrochemical Soc., 104, 397, 1957.
2. H. Schmalzried: z. f. Physicalische Chemie NF, 25, 178, 1960.
3. C. B. Alcock and T. N. Belford, Trans. Faraday Soc. 60, 822, 1964.
4. W. Pluschkell and H. Engel: J. Metallkunde, 56, (7), 450, 1965.
5. W. A. Fisher and W. Ackermann: Arch. f.d. Eisenhuttenw 36, 643, 1965.
6. M. Kolodney, B. Minushkin, and H. Steimnetz: Electrochem. Tech, 3, (9-10), 244, 1965.
7. Y. Matsushita and Goto: Thermodynamics IAEA (Vienna) 1, 1966.
8. T. C. Wilder: Trans Met. Soc. AIME, 236, 1035, 1966.
9. R. Baker and J. M. West: J. British Iron & Steel Inst., 204, 212, 1966.
10. E. T. Turkdogan and R. E. Fruehan: 76th General Meeting AISI, May, 1968.

In certain forms of my novel direct measurement apparatus, the probe structure can be enclosed with a self-contained oxygen-based reference material therein. This avoids the necessity of conducting air or other oxygen-containing material into the probe structure from an external source during use of the probe.

I accomplish the desirable results described heretofore and overcome the defects of the prior art by providing a probe capable of being plunged into a high temperature liquid metal without destructive thermal shock for the purpose of determining the dissolved oxygen content of said liquid metal, said probe comprising an elongated electrically insulating refractory envelope, a small mass of a refractory oxide-type oxygen-anion permeable solid electrolyte material supported adjacent one end of said envelope, at least a portion of at least one side of said mass being exposed through an opening in said envelope for contact with said liquid metal, said one side portion being disposed adjacent said one envelope end, reference means within said envelope for contacting an apposed side of said mass with an oxygen-reference material, and circuit means extending into said envelope for electrically contacting said apposed mass together with additional circuit means disposed for electrically contacting said liquid metal for measuring an emf developed across said mass

in proportion to the concentration of said dissolved oxygen in said liquid metal.

I also desirably provide a similar combination wherein said envelope is fabricated from a material selected from the group consisting from alumina, fused silica and fused quartz.

I also desirably provide a similar combination wherein said electrolyte material is an unsaturated oxide spinel-type crystalline material selected from the group consisting of materials conforming to the following general equations:



where *M* and *N* equal metals of dissimilar valances, and the oxide of the lower valence metal is present in less than the stoichiometric amount thereof.

I also desirably provide a similar combination wherein said reference means include a metal member positioned substantially against said apposed mass side, said member being fabricated from a metal which is oxidizable at the temperature of said liquid metal to an oxide capable of providing an appreciable equilibrium oxygen reference pressure at said temperature.

I also desirably provide a similar combination wherein said metal member includes a powdered mass of said metal.

I also desirably provide a similar combination wherein said metal member is relatively thin foil of said metal.

I also desirably provide a similar combination wherein said metal member includes an alloy of dissimilar metals capable of shifting the calibration curve of said probe.

I also desirably provide a similar combination wherein temperature sensing means are mounted within said envelope for measuring the temperature of said apposed mass side.

I also desirably provide a similar combination wherein said envelope is mounted on a support therefor, a cap member is removably mounted on said support, said cap member being shaped to enclose the otherwise exposed end of said envelope and said mass.

I also desirably provide a similar combination wherein said reference means are retained against said apposed mass side, an elongated electrically insulating tube is inserted through said envelope to a position of engagement with said reference means to retain said reference means against said mass, said tube forming passage means for conducting excess or residual gas out of said envelope.

These and other objects, features, and advantages of the invention, together with structural details thereof, will be elaborated upon as the following description of presently preferred embodiments and presently preferred methods of practicing the same proceeds.

In the accompanying drawings, I have shown presently preferred embodiments of the invention and have illustrated presently preferred methods of practicing the same, wherein:

FIG. 1 is a longitudinally sectioned view of one form of probe structure arranged in accordance with the invention;

FIG. 2 is a cross sectional view of the probe structure shown in FIG. 1 and taken along reference line II-II thereof;

FIG. 3 is an enlarged elevational view, partially sectioned, of one form of the insulating envelope and electrolyte pellet arrangement which can be utilized in the probe structures of FIGS. 2 and 4;

FIG. 4 is a partial longitudinally sectioned view of another form of probe structure arranged in accordance with the invention;

FIG. 5 is a partial longitudinally sectioned view of the probe structure of FIG. 4 and showing the probe structure in its extended, operative position with reference to the molten material being analyzed;

FIG. 6 is a graphical representation of the calibrated electrical output of my novel probe utilizing various types of oxygen-reference materials;

FIG. 7 is a partial, longitudinally sectioned view of still another form of my novel probe structure having self-contained oxygen-reference means;

FIG. 8 is a similar view showing still another form of my novel probe structure with self-contained oxygen-reference means in a partially sealed probe structure;

FIG. 9 is a similar view of another form of my novel probe structure having a combined electrode, electrode lead and oxygen-reference material within the probe structure;

FIG. 10 is an isometric view of still another form of my direct oxygen measurement apparatus;

FIG. 11 is a partial cross sectional view of still another form of my direct oxygen measuring apparatus shown in a unique arrangement with a continuous casting machine or the like;

FIG. 12 is a partial longitudinally sectioned view similar to FIG. 9 and showing a modified probe structure;

FIG. 13 is a similar view of still another form of my probe structure.

Referring now to FIGS. 1-2 of the drawings, the illustrative form of the probe structure 44 shown therein includes an envelope 46 fabricated from fused silica, alumina, or fused quartz or the like electrically insulating material which is sufficiently refractory and chemically resistant to withstand molten metal or other high temperature material for an interval at least sufficient to permit a reading to be made. In the case of molten steel analyses, fused silica or quartz is preferred. Fused silica has a melting point of about 1,710° C. and begins to soften at a temperature of about 1,650° C., which is higher than that of most liquid steels during refining. In any event, slight softening of the envelope 46 does not interfere with the reading, which is substantially instantaneous. Moreover, a rapid heating of the envelope to an elevated temperature, particularly one in the vicinity of its softening temperature, prevents cracking of the envelope by the mass 52 (described below), which may have a considerably higher coefficient of expansion. The relatively small sizes of the envelope 46 and mass 52 also mitigate the effects of their differing rates of thermal expansion. Proper selection of refractory materials is important since the probe may be used in liquid metals at elevated temperatures above 1,000° C. to include the complete range of melting temperatures of the wide variety of liquid steels, and other high temperature liquid metals, such as molten copper. More critically, in the case of certain electrolyte materials useful herein, a significant oxygen-ion conductance

does not occur until a temperature of about 800° C. is attained.

This envelope 46 in this example is retained in a length of iron tubing 48 or other suitable support, on the outer surface of which is supported an electrode 50, which is fabricated from an electrically conductive material capable of withstanding molten metal at elevated temperatures. The electrode 50, if desired, can be separated from the probe structure for independent insertion into the liquid metal. Of course, the iron tubing 48 itself can serve as the external electrode in place of the electrode 50. In any event, the electrode 50 can be shaped for coinsertion with the probe 44 to a predetermined depth in the liquid metal. Examples of such coinsertion are evident from FIGS. 10, 12, and 13 described below.

At the outward end of the envelope 46, a mass 52 of solid electrolyte material, such as one of the solid electrolytes described below, is retained as by melting or heat-forming the walls of the envelope 46 about the mass 52 or by sintering the mass 52 (in either pellet or pulverulent form) to the adjacent internal wall surfaces of the envelope 46 without appreciable forming of the envelope, as noted below. For maximum thermal resistance the mass 52, in any case, is of small size and compact of configuration, as evident from the drawings, particularly FIG. 3 (enlarged as aforesaid). A desirable configuration for the mass 52, as evident from FIGS. 1 and 3 and from FIGS. 7-9, 12 and 13, is right-cylindrical wherein the diameter and height of the cylinder are about equal. For operation of the probe, it is necessary only that the mass 52 be sealed to the envelope 46, to an extent to prevent leakage of liquid metal into or gas out of the probe.

In this example, a very reliable seal is produced as by heat-forming the envelope material about the mass 52. Heat-forming of the envelope can be accomplished by spinning or rotating the envelope about its longitudinal axis while heating at least that portion thereof adjacent the mass 52 to the softening point of the envelope material.

The seal results from a sintering action which inherently occurs when solid electrolyte and envelope materials of comparable sintering and softening temperature ranges are employed. For example, a zirconia-calcia mass 52 (or an electrolyte of similar melting point such as yttria-stabilized thoria) has a sintering temperature range of about 2,000° F. to about 3,000° F. and is inherently sintered to a fused silica envelope having a softening point of about 3,000°-3,100° F. Sintering occurs between the electrolyte mass 52 and the adjacent surface of the silica envelope to form an excellent ceramic-to-ceramic seal. In addition, individual particles of the mass 52 are sintered or resintered, as the case may be, to one another for increased strength and reduced porosity of the electrolyte mass 52. The probe 44 is highly resistant to thermal shock.

In one arrangement, the mass 52 can be provided in the form of a discrete pellet or disc to which the walls of the envelope 46 can be shaped thereabout, as shown in FIG. 1; or alternatively the pellet can be inserted into a length of tubing 46' (FIG. 3) made of the aforementioned insulating materials and having about the same inner diameter as the outer diameter of the mass 52'. In the latter case, the adjacent wall positions of the envelope 46' can be heat-formed and spun upon the outer

cylindrical periphery of the pellet 52' to form a seal therewith, as noted above.

In another arrangement the mass 52 can be inserted as a small bit of paste of a pulverulent solid electrolyte material in a suitable binder or agglutinant material such as a relatively small amount of colloidion.

In forming a powdered zirconia-containing electrolyte into a special shape, such as the mass or disc 52 in the end of the envelope 48, or other structure, such as the electrolyte insert of FIG. 12, I convert the powder into a paste or plastic mass by mixing it with the aforesaid agglutinants. Certain polymers, such as polyvinyl alcohol, carboxy methylcellulose and/or gum gatti in an aqueous solution, can also be used for this purpose. The agglutinant or binder aids in compacting the mass against the surface of the envelope, and thus improves the bond between the envelope and the electrolyte mass.

Zirconium citrate or other organic compound of zirconium also can be used. Upon heating the mass, in situ, in an oxidizing atmosphere, the zirconium compound binder is decomposed and  $ZrO_2$  is formed thus bonding the particles together. The mass then retains its shape when heated to high temperatures, such as in baking or sintering, or in subsequent use, and is rendered more impervious by this treatment.

The preparation of an oxygen sensor or probe which has a combination of chemical and physical properties for resisting destruction and malfunction when plunged into a high temperature liquid metal such as steel has been accomplished by at least two features of the invention which constitute essential bases for this invention.

The disclosed materials when combined not only 35 jointly withstand extreme thermal shock without shattering but also do not decompose or melt. In addition, the combination resists erosion and destructive chemical reaction or other contamination by the liquid metal or its dissolved oxide during such immersion. Failure of the probe to comply with any of these stipulations will result in either malfunction or an erroneous indication of the oxygen content of the material.

Thus, a primary feature of the invention is a proper selection of the materials for the envelope and the electrolyte. For example, fused silica when selected from 45 one of the envelope materials and calcia-stabilized zirconia when selected from one of the electrolytes exhibit these properties either individually or collectively in the proposed structure. A second primary feature involves a special sintering method for installing or inserting a mass of solid electrolyte into a fixed position at or near the end of a tubular envelope.

In this procedure, after certain preliminary steps depending upon whether a pellet or a powdered mass of electrolyte is being installed, the tip of the probe containing the electrolyte is heated to a temperature in the range of 2,000° F and preferably approaching 3,000° F.

The selected materials are sufficiently compatible so that they interact to form a secure bond. In the case of the combination of calcia-stabilized zirconia and a silica tube, the  $CaO$  of the electrolyte reacts with the  $SiO_2$  of the tube to form a film of calcium silicate at the interface, thus securely bonding the two materials. In the case of a probe structured with the calcia-stabilized zirconia in an alumina tube, for example, sintering results in a reaction between the  $CaO$  of the electrolyte and

the  $Al_2O_3$  of the tube to form an interfacial compound of a spinel configuration ( $CaAl_2O_4$ ).

Rapid cooling from the sintering temperature tends to stabilize the high temperature configuration so that 5 the thermal shock is greatly reduced when the probe is plunged into high temperature liquid metal.

Desirably, but not necessarily, the envelope material has a softening temperature range within the sintering range of the electrolyte material to facilitate sintering 10 and sealing thereof to the envelope, as noted previously.

The envelope 46, together with the mass 52 is releasably held in the probe structure 44 so that this portion of the assembly can be discarded after one or more 15 measurements. When using the probe 44, the forward surface of the mass 52 is exposed to the molten material through the otherwise open end of the envelope 46. Desirably, the forward surface of the mass 52 is adjacent the associated end of the envelope as shown. In 20 certain applications, however, the mass can project through the envelope opening. In most applications, on the other hand, the envelope opening, and in this case the I.D. of the tubular envelope, are kept small, so as to reduce that surface of the mass 52 which must be exposed to the liquid metal.

As is well-known, the coefficients of thermal expansion of many of the electrolyte materials disclosed herein are larger than those of the noted envelope materials. In those applications wherein the electrolyte coefficient is substantially larger, the effects of differential thermal expansion can be mitigated, when necessary, by heating the envelope, during use of the probe, at a very rapid rate from its initial temperature to the elevated temperature of the liquid metal and preferably by selecting an envelope material which begins to soften at the elevated temperature. The envelope, then, becomes slightly plastic before sufficient heat penetrates the walls thereof to the electrolyte to cause appreciable thermal expansion of the latter.

Oxygen reference means can be placed in the envelope 46 or 46' and desirably against the apposed surface of the mass 52 or 52'. The reference means can take the form of a metal foil or coating 54 or other metal member as described below. A cermet member, or an alloy can also be used. Oxygen from suitable oxygen-reference means such as those described below, diffuses readily through the coating. In the case of pure iron, for example, reference oxygen quickly saturates the iron foil before an oxidation commences. In other arrangements of my invention, the coating is provided as a piece of foil or other discrete member pressed or held against the mass 52 for contact purposes. Reference oxygen can then pass around as well as through the contact member.

Although the coating 54 facilitates intimate contact between the mass 52 and an electrical connection such as thermocouple 56, the coating is not essential as pointed out below. The electrode coating can be replaced by a discrete electrically conductive member or mass held against the electrolyte member 52, for example, by the elongated member 60 mentioned below. The electrode coating or member 54 can be combined with or serve additionally as a solid oxygen reference means, as also noted below. The thermocouple 56, in this example, also provides an electrical connection to the opposite or other apposed surface of the mass 52 through one of its leads, for example, the lead 58. The

other electrical connection can be provided by lead 51 and electrode 50, since the envelope 46 is of insulating material.

The thermocouple leads 58 and 59 are insulated and conducted through the envelope 56 to the thermocouple 56 by suitable means such as an apertured and elongated insulating member 60, fabricated like the envelope 46 from fused silica, alumina, quartz or the like. The insulating member 60 desirably is spacedly fitted within the envelope 56, and is provided with a pair of longitudinally extending, laterally spaced apertures 62 through which the thermocouple leads 58, 59 are loosely extended. The passages 62 therefore can provide access for external air or other oxygen-containing gas to the thermocouple side of the electrolyte disc 52. Desirably, the member 60 presses the thermocouple 56 into good electrical and thermal contact with the mass 52, and with a discrete electrode and/or oxygen reference member when used. In this relation, the member 60 can be affixed after the teaching of FIG. 9, for example.

Other oxygen containing materials such as  $\text{CO}_2$  or various cermets, (and many other oxygen-bearing compounds some of which are noted hereinafter) can be used as oxygen-reference means. These materials dissociate at the elevated temperatures to which the probe usually is subjected as follows:



As such compounds have differing dissociation energies, the probe usually requires calibration for each such source of oxygen.

The aforementioned reference gas can be circulated inwardly through the rod apertures 62 to the inner surface of the pellet 52 and then outwardly through clearances 63 between the rod 60 and the envelope 46 as denoted by flow arrows 65. On the other hand, the rod 60 can be closely fitted within the envelope 46 and a central longitudinally extending baffle (not shown) can be utilized to circulate a reference gas forwardly through one of the passages 62 and in the return direction through the other passage 62.

It has been found that ready access of the inner surface of the solid electrolyte disc 52 to a standard oxygen-reference source is necessary in order to obtain a prompt reading of stabilized emf output from the probe, when the molten material contacts both the mass 52 and the electrode 50. In one arrangement of my oxygen-reference means, a steady but not necessarily strong flow of reference gas is thus maintained. In fact, still air has been used as a reference material. It is contemplated that the quantity or concentration of oxygen available from the oxygen-reference means can be varied as noted below or by adding a quantity of nitrogen or other relatively inert gas, so as to shift the calibration curve of the electrolyte cell to another, more easily measured potential range (FIG. 6).

It will be understood, of course, that the use of the thermocouple 56, and one of its leads, such as the lead 59, are not essential to the operation of the probe structure 44 and can be omitted, particularly if other temperature measuring means are available. Upon omission, the lead 58 will be connected directly to the inner coating or the like of electrode member 54 of the elec-

trolyte mass 52 in order to ensure the necessary electrical contact therewith. The aforementioned electrically conductive coating or member 54 is not essential, but is useful in facilitating electrical contact with the lead 51 or leads 58, 59 by pressure contact for example. Also, one of the gas and conductor passages 62 can likewise be omitted and the aforementioned circulation of oxygen-bearing gas can be returned through the clearances 63. The leads can be of very small diameter, so as not to obstruct the flow of an oxygen-reference gas, when used.

The mass 52 is sufficiently small, in this example, that any differential expansion between the solid electrolyte material comprising the mass 52 and the material of the envelope 46 will not cause the latter to fracture. In fact, the small size of the probe structure does not interfere with the electro-chemical aspects of its operation, and the probe can be "miniaturized", if desired, to an extent consistent with manufacturing techniques.

A further advantage of the structure of FIGS. 1-3 lies in the fact that the size and shape of mass 52 considerably reduces the cost of manufacturing the probe structure 44, as compared to the case where the entire envelope 46 or a substantial portion thereof is fabricated from the solid electrolyte, which is a rather expensive material. The latter advantage is an important consideration in view of the fact that the electrolyte mass 52 and the envelope 46 in many applications must be replaced in the probe structure 44 after each reading particularly after insertion into high temperature liquid metals, such as molten steel. The expendable envelope 46 and mass 52 together represent a small fraction of the cost of fabricating the entire envelope from an electrolyte material. The latter envelope, even if it does not fracture from thermal shock, must also be expended after each use, which renders the cost thereof prohibitive for most applications.

Referring now to FIGS. 4 and 5 of the drawings, wherein similar reference characters with primed accents denote similar components of FIGS. 1 and 2, another probe structure 70, arranged in accordance with the invention, is illustrated. The latter arrangement is adapted particularly for determining oxygen content of a liquid metal in most refining furnaces, such as the open hearth, where it is necessary to protect the probe from contact with an overlying layer of molten slag thereon as the probe is immersed below the slag-metal interface. Thus, the probe structure 70 is provided with means for shielding the solid electrolyte from contact with the overlying slag layer and for quickly inserting the probe components into the molten bath in order to obtain a stabilized reading.

In furtherance of these purposes, the supporting envelope 44' together with the electrolyte mass 52' secured therewith are mounted in a plug member 72, through which the envelope 44' is extended centrally and longitudinally. The plug 72 is inserted into a central and longitudinally extending channel 74 of a tubular electrode 76 fabricated from a compatible material such as steel. Electrical contact to the tubular electrode 76 and to the electrolyte disc 52' is established by lead 51' and one of the thermocouple leads 58' or 59' as described above in connection with FIGS. 4 and 5. An oxygen reference gas, such as air or  $\text{CO}_2$ , can be circulated to the inner surface of the disc 52' and/or the thermocouple 56' can be eliminated as described previously with reference to FIGS. 4 and 5.

The tubular electrode 76 and the components of the probe structure 70 supported thereby, are slidably mounted within an outer supporting tube 82, likewise fabricated from a compatible material insofar as the material being tested is concerned. The tubular electrode 76 is thus mounted for movement longitudinally of the outer support tube 82, and in this example is secured to the adjacent end of a compressed resilient member such as a coil spring 84. The spring 84 is maintained in its compressed condition in this example by a pin 86 inserted through a suitable aperture in the support tube 82 and movable laterally to restrain and to release the compressed spring 84, as required. In the probe structure 70 as shown in FIG. 4 4 the pin 86 engages the next to the last helix of the coil spring 84 to maintain the major proportion of the spring 84 in its compressed condition and the tubular electrode 76 and associated components in their inoperative position in the outer support 82.

In this position, the insertable ends of the tubular electrode 76 and of the envelope 44' and disc 52' are covered by a removable cap 88, which can be frictionally or otherwise detachably secured to the adjacent end of the outer support tube 82 by suitable quick fastening means (not shown) secured to the outer flange 90 of the cap and the adjacent end 92 of the support tube 82. The inward end of tubular portion 94 of the cap 88 is of sufficient length to engage the adjacent end of the tubular electrode 76 in this position.

In the operation of the probe structure 70, the lower end of the support tube 82, as viewed in the drawings, is inserted through any overlying slag and well into the molten steel or other material to be analyzed. The pin 86 is then withdrawn, for example by means of its eye-hook 96, to release the ejection spring 84. The slidably mounted tubular electrode 76 carrying with it the envelope 44' and electrolyte disc 52' and the detachable cap 88, is then ejected downwardly farther into the molten steel or other liquid metal, where it comes to rest at the extended position of the ejection spring 84 as shown in FIG. 5 of the drawings. The inserted movement of the probe forces the protective metal cap 88 into the metal where it dissolves or melts or falls away to allow normal use of the probe. While in place, the cap 88 prevents contact of the molten slag and concomitant erroneous readings caused by coating of the slag on the ejected components of the probe structure 70. At the fully extended position of the probe structure (FIG. 4), the relatively small exterior surface of the solid electrolyte disc 52' and the tubular electrode 76 thereto are exposed to the substance being measured at a predetermined depth.

The electrolyte mass 52 or 52' desirably is fabricated from a suitable solid material which resists melting at any anticipated elevated temperature and exhibits solid electrolytic properties. In those applications involving the testing of molten steel, where high oxygen content with relatively low percentages of carbon, silicon, and alloying constituents are anticipated, the electrolyte mass can be made from zirconia stabilized with calcia, as noted above. In applications involving other high-melting liquid metals, stabilized zirconia or thoria, for example, can be used to advantage.

In general, combinations of oxides can be utilized which exhibit electrolytic properties by providing the necessary defects in the crystalline lattice which allow the transport of oxygen ions. Principal among these are

partially saturated complex oxides, which otherwise conform generally to the spinel-type crystalline structure. Spinel type structures, for this purpose, are approximated by the generalized formula  $(MN_2O_4)$ , which results from at least three different combinations, as set forth generally in the following Table I. The most common spinel involves the combination of a monoxide with a sesquioxide, such as  $MgO$  plus  $Al_2O_3$  yielding an unsaturated  $MgAl_2O_4$ , when combined in non-stoichiometric amounts as described below. Other complexing procedures involve a dioxide and two molecules of monoxide, such as  $2CaO + ZrO_2 = ZrCa_2O_4$ , and a trioxide with a suboxide for example  $Cu_2O + WO_3 = WCu_2O_4$ . It will be seen that substantially the same molecular structure results regardless of the particular forms of oxide combinations involved. These spinel type compounds can exhibit similarly unsaturated crystalline structures.

There are large numbers of other oxide complexes which fall into one of the types of oxide complexes noted above and which form spinel-type molecular structures. Some of these are noted in the following table:

TABLE I TYPES OF SPINELS

| TYPE I                       | TYPE II                     | TYPE III                    |
|------------------------------|-----------------------------|-----------------------------|
| $MO_2N_2O_4$ or<br>$MN_2O_4$ | $2 MO.NO_2$ or<br>$NM_2O_4$ | $M_2O.NO_2$ or<br>$NM_2O_4$ |
| $MgAl_2O_4$                  | $FeCr_2O_4$                 | $TiMg_2O_4$                 |
| $MgCr_2O_4$                  | $NiCr_2O_4$                 | $ZrMg_2O_4$                 |
| $MgFe_2O_4$                  | $CuCr_2O_4$                 | $CbMg_2O_4$                 |
| $CaAl_2O_4$                  | $ZnCr_2O_4$                 | $TaMg_2O_4$                 |
| $MnAl_2O_4$                  | $CbCr_2O_4$                 | $TaNi_2O_4$                 |
| $FeAl_2O_4$                  | $CdCr_2O_4$                 | $TiCa_2O_4$                 |
| $CoAl_2O_4$                  | $CoFe_2O_4$                 | $CbZn_2O_4$                 |
| $NiAl_2O_4$                  | $MnFe_2O_4$                 | $TaZn_2O_4$                 |
| $ZnAl_2O_4$                  | $FeFe_2O_4$                 | $ZrCr_2O_4$                 |
| $ChAl_2O_4$                  | $NiFe_2O_4$                 | $TiMn_2O_4$                 |
| $CdAl_2O_4$                  | $ZnFe_2O_4$                 | $TaCr_2O_4$                 |
| $CaCr_2O_4$                  | $MgV_2O_4$                  | $TiFe_2O_4$                 |
| $CaFe_2O_4$                  | $FeV_2O_4$                  | $TiCd_2O_4$                 |
| $CoCr_2O_4$                  | $ZnV_2O_4$                  | $TiCo_2O_4$                 |
| $MnCr_2O_4$                  |                             | $UFc_2O_4$                  |
|                              |                             | $TiZn_2O_4$                 |
|                              |                             | $UNi_2O_4$                  |
|                              |                             | $ZrMn_2O_4$                 |
|                              |                             | $UZn_2O_4$                  |
|                              |                             | $CbMn_2O_4$                 |
|                              |                             | $UCb_2O_4$                  |
|                              |                             | $TaMn_2O_4$                 |
|                              |                             | $UCd_2O_4$                  |
|                              |                             | $ZrFe_2O_4$                 |
|                              |                             | $VMg_2O_4$                  |
|                              |                             | $CbFe_2O_4$                 |
|                              |                             | $VZn_2O_4$                  |

However, in order to be used for solid electrolytes one of the constituent oxides must be present in less than the stoichiometric amount to permit the formation of the ion transport defects in the crystalline lattice. For example, in the monoxide-dioxide spinel formation, such as  $ZrCa_2O_4$ , 15 mol percent of calcium oxide rather than the theoretical 66 percent is used, to produce an unsaturated spinel lattice. The unsaturating percentage of the stabilizing oxide will, of course, vary depending upon the particular oxide complex which is used.

Complex oxide combinations can be employed other than typically spinel-type structures. For example, an oxide complex formed from a dioxide and a sesquioxide, such as  $ThO_2 + Y_2O_3 = ThY_2O_5$ , exhibits electrolytic properties in the non-stoichiometric condition. The essential requirement of the electrolytic complex oxide combination is that one of the complexing oxides be present in a non-stoichiometric amount to provide the necessary crystalline lattice defects (oxygen vacancies) and resulting oxygen ion transference. By this mechanism, the unsaturated oxide complex from which the mass 52 or 52' is formed, develops an emf equivalent to the differential in oxygen concentration at the apposed sides or surfaces thereof. A suitable meter can

be calibrated to read the *emf* output of the probe in terms of oxygen concentrations in the material whose oxygen content is unknown at one side of the mass. Such calibration of course will be related to a given known oxygen concentration at the other mass side.

FIG. 6 of the drawings is a logarithmic graph showing the variation of probe emf in millivolts with concentration of dissolved oxygen in parts per million. The illustrated curves for various types of oxygen-reference materials were obtained in molten steel at 2,900° F. The least desirable of these reference materials is air, as denoted by curve 110, which exhibits relatively high voltage requiring special instrumentation and in some cases causing the electrolyte to break down. Curve 112, representing the use of  $\text{CO}_2$  is of special interest, on the other hand, owing to its substantially greater slope and lower voltage.

Except as provided by my invention, the use of  $\text{CO}_2$  or other gaseous material as an oxygen reference entails the continuous circulation of the gas through the probe structure. I avoid such continuous circulation while preserving the advantage of a higher  $\Delta\text{emf}/\Delta O$  characteristic from the use of a  $\text{CO}_2$  reference, with the self-contained feature of FIG. 8 or 9 described below.

A number of cermet-like materials for example  $\text{Ni-NiO}$ ,  $\text{Fe-Fe}_x\text{O}$ ,  $\text{Cr-Cr}_2\text{O}_3$ ,  $\text{W-WO}_2$ ,  $\text{Co-CoO}$ ,  $\text{Cb-CbO}_2$ ,  $\text{Mo-MoO}_2$ , and various other oxidizable metals and their oxides have been proposed for use with known solid electrolyte structures. These cermets, which desirably contain a preponderance of free metal for the purposes of the present invention, are especially advantageous when used in my novel probe structure, since their electrical conductivities permit electrical contact with the mass 52 therethrough. To qualify for such usage, the cermet including the free metal and its oxide must be sufficiently refractory at the anticipated operating temperature range of the liquid metal or other material to be measured. There must be no undue vaporization of the oxide but there must be a discernible equilibrium oxygen-pressure at the operating temperature range.

The emfs obtained with some of these materials are represented by curves 114, 116 and 118. The  $\text{Ni-NiO}$  and  $\text{Fe-Fe}_x\text{O}$  curves 114, 116 are satisfactory for certain applications. However, the  $\text{Cr-Cr}_2\text{O}_3$  curve 118 crosses the zero emf line at point 120 with the result that concentrations of dissolved oxygen in the range of 20-50 ppm are very difficult to measure. These and other oxygen-reference materials can be utilized, including the disclosed oxygen-reference means described below.

I have found that the addition of a dissimilar metal to the aforementioned cermet-like materials displaces the *emf* curve, as typified by curve 122 for the oxygen-reference material,  $\text{NiCr-Cr}_2\text{O}_3$ . This material which is a combination of nichrome and chromium oxide displaces the undesirable curve 118 to the left and away from the zero emf line 124. The curve 122 has the additional advantage that the *emf* varies directly with dissolved oxygen concentration. The calibrational curves of the other cermet materials can be similarly displaced. It appears that a more noble metal shifts the *emf* curve as a function of the activity of the diluent metal.

In FIG. 7 of the drawings, another arrangement 126 of my novel direct measurement apparatus is shown. In this example oxygen measuring probe 128 is inserted

through a refractory holder 130. The probe 128 and the block 130 are supported by a length of steel or other metal tubing 132. A small mass of solid electrolyte 136 is sealed into an insulating tube 128 of the probe structure 138 by one of the methods described above.

A combined electrode and oxygen-reference member including in this example of relatively pure foil 140 of an oxidizable metal is supported against the inner surface 142 of the electrolyte 136. The member 140 can be backed up by a metal foil or disc 144, or other noble metal. Electrical contact is made with a length of conductive wire 146 which can be made of platinum. The wire 146 is supported at the other end of the insulating tube 138 by means of refractory cement 148. If desired, a suitable insulating tube, as in FIG. 8, can be used to press the wire 146 against the member 144 if used and the electrode oxygen reference member 140 or similar metallic member and in turn against the adjacent surface 142 of the electrolyte 146. I have found that such pressure is sufficient to establish proper electrical contact between the lead 146 and the solid electrolyte 136.

The small bit of foil or other member 140, which can be made from an oxidizable metal such as iron, chromium, nickel, cobalt, molybdenum, tungsten or columbium, provides the oxygen based reference material for the proper operation of the electrolyte cell. Thus, a small amount of air or other form of gaseous oxygen contained within the interior 150 of the probe 128, is sufficient to form a very thin layer of oxide on the member or foil 140. The amount of the oxide layer is increased by the passage of oxygen ions through the solid electrolyte 136 when the probe 126 is immersed. I have found that the amount of oxide thus formed within the envelope 128 is sufficient to attain an equilibrium and reproducible *emf* reading. The addition of a more noble but oxidizable dissimilar metal to the reference foil or member 140 likewise shifts the calibrational *emf* curve as shown in FIG. 6. For example, a disc 140 formed from nichrome shifts the calibration curve to the left relative to the curve for a pure chromium disc 140, after the manner illustrated in FIG. 6.

A layer or tube of protective cardboard 142 or other refractory material surrounds the outer surfaces of at least that part of the supporting tube or holder 132 which may be immersed in the molten metal bath or the like. The exposed surface 154 of the electrolyte 136 is protected during its passage through any slag or other overlying layer on the bath or heat by means of a suitably shaped cap 156, which can frictionally engage the adjacent end of the cardboard layer 152. For use with molten steels the cap 156 can be fabricated from a mild steel which is quickly melted to expose the electrolyte surface 154 at some point or predetermined location beneath the surface of the steel bath.

As mentioned in certain of the preceding figures, it will be understood, of course, that a second lead (not shown in FIG. 7) can be introduced into the insulating tube or envelope 128 for the purpose of making a thermocouple connection at the electrode member 140 or 144. It is also contemplated that the electrode and reference member 140 can be replaced with a mixed metal or alloy member such as a piece of nichrome. As set forth in FIG. 6, I have found that the use of a nichrome foil displaces the *emf* calibration curve to a more favorable position (curve 122) relative to that ob-

tained with chromium (curve 118). Similar alloys can be employed to fabricate the member or foil 140 to displace the various calibration curves more or less at will.

In construction of the probe 126 of FIG. 7 it is not necessary that the member or foil 140 be sufficiently refractory to withstand melting at the operating temperatures of the probe 126. For example, I have obtained equally good results from the use of a pure iron foil 140 or other metal which melts within the operating temperature range of most liquid steels. For this reason, the foil or other oxidizable metallic member 140 can be provided in the form of particulate or pulverulent material.

Carbon or graphite can be substituted for the oxygen-reference means 140 after the teaching of FIG. 7. It is also contemplated that a suitable electrically conductive and self-contained oxygen reference material such as cermet, can be substituted for the member 140. The cermet, which can be selected from those materials enumerated or characterized in connection with FIG. 6, is provided as a suitable member or mass positioned against and hence in electrical contact with the solid electrolyte mass 52. The cermet, for this purpose, therefore can be provided in the form of a foil or other discrete member, or as a pulverulent mass. Either form may be pressed against the solid electrolyte 52 as by use of the contact foil or disc 144 or similar contact, or, operating conditions permitting, by gravity. Where the mass of reference material 140 is a discrete member and is sufficiently refractory to withstand melting at the anticipated operating temperatures, the contact member 144 can be omitted and electrical contact made directly to the reference member 140.

In FIGS. 8 and 9, I provide convenient means for generating carbon dioxide ( $CO_2$ ) within the probe structure as an oxygen-reference material. The desirability of using  $CO_2$  has been established in connection with FIG. 6. As explained more fully hereinafter, the probe structure 158 of FIG. 8 can be partially closed, while the probe structure 160 of FIG. 9 is closed but not sealed. The probe structures 158, 160, as is the case of the structure 128 of FIG. 7, can be employed as part of the measuring apparatus 126 or 126' (FIGS. 7 and 8). The probe support 126 may be plunged manually into the molten steel bath or the like, with the provision of a probe support 126 of suitable length, for example, as used in connection with a conventional immersion thermocouple. It is also contemplated that the immersion gun structure of FIGS. 4 and 5 can be used.

With more particular reference to FIG. 8, the solid electrolyte 136' is supported in insulating tube 138' in the manner described previously. Electrical contact can be established with the inner surface 142' of the electrolyte 136' by means of a conductive wire lead 162 or the like. Electrical contact between the wire lead 162 and the electrolyte surface 142' can be established as shown in FIG. 1. However, I have found, in most cases, that the platinum or other metallic coating can be omitted from the surface 142', and adequate electrical contact can be made between the electrical lead and the electrolyte by merely pressing these components together. In one arrangement, this is accomplished as shown in FIG. 9 by forming an enlarged contact portion 164 adjacent the inner end of the lead 162. An inner insulating tube 166 is then furnished for the purpose of engaging and pressing the spiral 164 into firm contact with the electrolyte surface 142'. Alterna-

tively, the lead is simply bent over the inward end of the inner tube 166. This engagement is preserved by securing the adjacent surface of the inner tube 166 to the other end of the probe tube 138' by means of a refractory cement 168. Alternatively, the inner end of the lead can be embedded in the electrolyte mass, particularly when the latter is supplied as a bit of pulverulent material.

In further accordance with my disclosure of FIG. 8, I provide a solid oxygen reference material 174 preferably within the space 172 between the inner or lead supporting tube 166 and the outer electrolyte supporting tube 138'. The material 174 is conveniently coated on the outer surfaces of the inner tube 166 and is capable of releasing an oxygen reference gas at elevated temperatures for the proper operation of the electrolyte cell 136'. As an example of such material 174, I use magnesium carbonate ( $MgCO_3$ ) or manganese carbonate ( $MnCO_3$ ), or preferably calcium carbonate ( $CaCO_3$ ), which decompose to release carbon dioxide ( $CO_2$ ) at the respective operating temperatures of the probe 158. In this arrangement, the outer end 170 of the inner tube 166 is left open. As the material 174 decomposes, the liberated  $CO_2$  or other oxygen reference gas travels toward the electrolyte 136' and comes into intimate contact with the inner surface 142' thereof, owing to the close proximity of the inner end 176 of the inner tube 166. For use in measuring the dissolved oxygen content of liquid steels, the inner insulating tube 166 desirably is fabricated from fused silica or quartz or alumina as is the electrolyte supporting tube 138'. The probe structure 158 is not sealed, and it possesses the advantage of producing a very quick, equilibrium reading, owing to the copious supply of  $CO_2$  from the decomposition of the rather limited quantity of material 174. A more obvious advantage is, of course, the elimination of an external source of  $CO_2$  and its attendant conduit connections, metering valves, etc.

A similar measuring apparatus 126' is shown in FIG. 9. The probe structure 160 used therein incorporates the advantageous use of CO (in the presence of carbon) to provide an oxygen reference within the probe. The inner surface 142' of the solid electrolyte is contacted by combined electrode, electrode lead, and oxygen reference member 178. In this example, the member 178 is a carbon or graphite rod extending substantially through the insulating tube 138' and is pressed at its inner end 180 to contact with the inner surface 142' of the electrolyte 136'. This relation, which produces adequate electrical conductivity between the electrode 178 and the electrolyte 136', is maintained by a rigid portion 182 of refractory cement or the like, positioned between the outer end 184 of the electrolyte supporting tube 138' and the adjacent surface of the electrode 178. The cement 182, however, can be porous or otherwise provided with a passage for the escape of air or gas when the probe 160 is heated.

When the other end, i.e., the electrolyte end of the insulating tube 138' is plunged into a bath of molten metal, the adjacent end 180 of the electrode 178 naturally attains the highest temperature along its length. At this time, the end portion 180 of the electrode quickly combines with air or oxygen contained within the insulating tube 138' to form carbon monoxide (CO) to yield a standard oxygen reference base for the probe 160. Thus, different forms of oxygen reference means

are produced in accordance with the following equilibrium reaction:



It is also contemplated that the rod can be made of other conductive and oxidizable or partially oxidized materials, to provide differing characteristics of the combined electrode, oxygen reference means, and electrical lead or conductor. Thus, the rod 178 can be fabricated with any of the cermet materials enumerated or characterized in connection with FIG. 6 or in connection with the conductive, oxygen-reference mass or member 140 of FIG. 7.

Another novel arrangement of my direct oxygen measuring apparatus 184 is shown in FIG. 10. The apparatus includes a refractory mold structure 186 through a wall section 188 of which are inserted an oxygen probe 190 and electrode 192. The probe 190 can be constructed in accordance with the insulating tube and electrolyte assembly shown in any of the preceding figures. Desirably, the probe 190 is one of the self-contained probe structures 128, 158, or 160 of FIGS. 7-9 for ready portability of the measuring apparatus 184. Suitable electric leads 194, 196 are connected to the probe 190 and to the exterior electrode 196 and thence to external emf measuring circuitry (not shown) of known construction. Although the material of the mold 186 is of an insulating character, it is not necessary, of course, to provide any particular means of insulating the electrode 192 from the probe structure 190, owing to the use of an insulating supporting tube 198.

In the operation of the direct measuring apparatus 184, a quantity of molten steel or other material having a temperature of at least 800° C and desirably 1,000° C or higher is poured into the mold 186 from a suitable ladle or spoon 200. The mold 186 is filled until the surface 202 of the molten material covers the probe 190 and the electrode 192. Electrical contact is established with the outer surface 204 of the solid electrolyte mass 206 through the molten steel 202 or the like and the external electrode 192. On the other hand, the inner surface 208 of the electrolyte mass 206 is contacted by means of the electrical lead 194. As noted below respecting FIG. 11, a thermocouple can be associated with the probe 190 in FIG. 10 for correlation with the *emf* reading of the probe 190. Desirably, the probe *emf* is measured at the solidification temperature of the liquid metal, as denoted by the temperature thereof becoming essentially constant. In the case of liquid steel, the melting temperature of specific alloys thereof can be quickly determined along with percentages of certain constituents such as carbon. The constant or freezing temperature thus obtained can be correlated with the *emf* of the probe to determine oxygen content.

In FIG. 11 another modification 210 of my novel direct measuring apparatus for dissolved oxygen is disclosed. In this arrangement, my apparatus is incorporated in a tundish 212 of a continuous casting machine, or in other suitable container structure, and is thereby enabled to perform a continuous monitoring of the oxygen content in the liquid steel passing through the tundish. Specifically I provide a stabilized zirconia (CaO · ZrO<sub>2</sub>) insert 214 for one or more of the nozzle openings, such as the opening 216 of the tundish 212. One of the other solid electrolyte materials listed above can be substituted for the stabilized zirconia, provided its

melting or softening point is above the anticipated temperature of the liquid steel.

The electrolyte insert 214 is contacted with an external measuring circuit and with an oxygen reference material to complete the electrolyte cell established by the insert 214. One arrangement for establishing such contact includes the provision of an insulating tube 218 extended through a conventional refractory wall structure 220 of the tundish 212. In this arrangement, a pair of electric leads 222 are extended through the insulating tube 218 and terminate in a thermocouple connection 224, which in turn is closely fitted into an adjacent recess 226 of the electrolyte insert 214 for electrical and thermal contact therewith. Alternatively, the thermocouple can simply be pressed against the bottom of the tube recess 227 in the insert 214.

Suitable oxygen reference material such as air or CO<sub>2</sub> from a suitable external source (not shown) can be conducted through the insulating tube 218 as denoted by flow arrow 228 to the inner end 230 of the insulating tube 218 where the reference gas contacts the adjacent surface of the electrolyte insert 214. The reference gas can then be conducted out of the insulating tube 218 through an inner tube 232 surrounding the leads 222.

As noted below, other oxygen reference means can be substituted.

Electrical contact with the inner surface or throat 234 of the electrolyte insert 214 is established through the liquid steel in the tundish 212 and through any metallic component of the continuous casting machine which is in contact with the liquid steel. To facilitate such contact, an external electrode 236 can be sealed through the wall structure 220 of the tundish 212 or inserted directly into the liquid metal through the open top of the tundish.

With this arrangement, an oxygen reference material can be continuously supplied to one side of the electrolyte insert 214 and a material of unknown oxygen content to the other side. The *emf* developed thereacross is continuously monitored by measuring the potential developed across external electrode lead 238 and one of the thermocouple leads 222. Owing to the rapid response of the direct measuring apparatus 210, a continuous reading of the dissolved oxygen content of the liquid metal passing through the electrolyte insert 214 can be obtained. Such readings can be calibrated against any changes of temperature, which are of course continuously indicated by the thermocouple 224. It will be appreciated that other suitable oxygen-reference means, such as one of those described above, can be substituted depending upon the specific application of the invention.

In FIG. 12 of the drawings, there is disclosed another form 240 of my novel probe structure which can be immersed or submerged below the surface of a liquid metal bath for simultaneously measuring the temperature and the dissolved oxygen content of the metal bath. The supporting tubing 242 as noted above in connection with FIG. 7 can be of any desired length for insertion manually lance-wise or with an ejection device into the metal bath. The tube 243 is protected in this example by a thermally insulating jacket 152' to which is fitted a protective cap 156'. Alternatively, the cap 156' can be engaged with the plug 248 or other common support for the probe and external electrode. A direct reading oxygen probe 244 and an external electrode 246 such as a rod of steel or other compatible

conductive material are inserted through suitable openings therefor in a refractory plug 248. In this example, the plug 248 can be secured to the end of the supporting tube 242 after the manner of FIG. 7.

A mass of electrolyte 250 is maintained within the exposed end of the insulating envelope 244 as described previously. The probe structure 244 can be fabricated as described in connection with any of the preceding figures, and, in this example, is provided with a thermocouple 252 positioned against an oxygen reference member 254 and the inside surface of the mass 250. Thermocouple and electrolyte leads 256 are extended through the interior of the envelope 244. As in other figures of the drawings, the refractory cement at the end of the envelope 244 merely stabilizes the leads 256 but does not seal the envelope. A similar lead 258 is connected to the external electrode 246, and all of the leads 256, 258 are extended through the supporting tube 242 for connection to external emf measuring circuitry (not shown). With the arrangement of FIG. 12 both the probe structure 244 and the external electrode 246 can be immersed beneath the surface of a liquid metal bath to the same predetermined depth, for measuring the dissolved oxygen content at that location. Substantially at the same time, the temperature at that location can be measured through the thermocouple 252.

A similar immersion and direct-reading probe 260 is shown in FIG. 13. In this arrangement the probe 244' and external electrode 246' are supported by a refractory block or plug 262. At the forward end of the plug 262, the protective cap 156' is engaged as in preceding figures. As noted previously the cap 156 or 156' can be used to prevent contact of the probe 244' with any overlying slag. By the same token, the cap 156 or 156' can be employed to prevent contact with the liquid metal until the forward ends of the probe and electrode can be immersed to a predetermined depth below the surface of the liquid metal.

In this example, the refractory block 262 is provided with a necked down portion 266 covered with an insulating layer 267 to which is secured an elongated supporting tube 268. Desirably, the supporting tube 268 is fabricated from a suitable structural material and is provided with longitudinally spaced commutator rings 269. The external electrode 246 is connected through lead 270 to contact 272 extending through the insulating layer 267, which can be of polyvinyl acetyl or the like for engagement with one of the commutator rings 269.

A pair of additional leads 274 for the thermocouple 252' are extended through the plug 262 to similar contacts 273 which are longitudinally spaced along the plug neck 266 for respective engagement with the remainder of the commutator rings 269.

The plug 262 together with the probe 244' and electrode 246', can be snapped into the supporting tube 268 by groove and detent means 275, 276. When thus engaged, the contacts 272, 273 are respectively engaged with the commutator rings 269, irrespective of the rotated position of the plug relative to the supporting tube 268. The rings 269 are connected to suitable leads 278 extended through the supporting tube 268. At least the forward end of the tube 268 is afforded a protective layer 280 of cardboard or the like such as a ceramic material. Desirably, the length of the insulation 280 is at least equivalent to the thickness of an overlying

ing slag layer (not shown) on a melt of liquid metal. Preferably, however, the length of insulation 280 exceeds such minimal length as the probe may be inserted to more than a minimal depth below the slag layer.

5 A suitable vent 282 is provided to relieve internal pressures when the probe 260 is heated.

From the foregoing, it will be apparent that novel and efficient forms of methods and means for determining oxygen content of materials have been described herein. While I have shown and described certain presently preferred embodiments of the invention and have illustrated presently preferred methods of practicing the same, it is to be distinctly understood that the invention is not limited thereto but may be otherwise variously embodied and practiced with the spirit and scope of the invention.

I claim:

1. A probe for determining the dissolved oxygen content of a high temperature liquid metal, said probe being capable of being plunged directly into liquid steel without destructive thermal shock, said probe comprising an elongated electrically insulating refractory envelope, a small mass of oxygen-ion permeable solid electrolyte material supported near one end of said envelope to seal said end of said envelope, at least a portion of the outer side of said mass being exposed through an opening in said envelope for contact with said liquid metal, means to provide an oxygen reference material in contact with the inner side of said mass, circuit means including a conductor extending into said envelope, and a second conductor disposed for contacting said liquid metal, said circuit means cooperating with said second conductor to measure an emf developed across said mass in proportion to the concentration of said dissolved oxygen in said liquid metal.

2. The probe according to claim 1 further including a thermocouple for measuring the temperature of said liquid metal and for correlation with said probe emf, said thermocouple forming part of said circuit means.

3. The probe according to claim 1 further including means for measuring the temperature of said liquid metal.

4. The probe according to claim 1 wherein said envelope is fabricated from alumina.

5. The probe according to claim 1 wherein said envelope is fabricated from either fused silica or from fused quartz.

6. The probe according to claim 1 wherein said electrolyte material is an unsaturated oxide-spinel type crystalline material selected from a group conforming to the following general equations:



where  $M$  is a metal of lower valence than metal  $N$  and is present in less than the stoichiometric amount to form the saturated spinel thereof.

7. The probe according to claim 1 wherein said electrolyte is selected from a group consisting of stabilized zirconia and stabilized thoria.

8. The probe according to claim 1 wherein said electrolyte material is calcia-stabilized zirconia and said envelope is fabricated from alumina.

9. The probe according to claim 1 wherein said electrolyte material is calcia-stabilized zirconia and said envelope is fabricated from fused quartz.

10. The probe according to claim 1 wherein said means to provide an oxygen reference material includes means for circulating an oxygen containing reference gas continuously through said probe.

11. The probe according to claim 1 wherein said envelope is mounted on a support, and said second conductor is substantially coterminous with said envelope to facilitate the determination of said oxygen content at a given location within said liquid metal.

12. The probe according to claim 1 wherein said second conductor has a tubular shape, and said probe further includes means for mounting said envelope generally within said tubular conductor.

13. The probe according to claim 1 further including an elongated support and a plug member, said envelope being mounted on said plug member which is detachably mounted on said elongated support.

14. The probe according to claim 13 wherein said plug member and said elongated support include interfitting portions respectively, and mating contact members disposed respectively on said interfitting portions,

said circuit means being connected to said plug member contacts, and external measuring circuitry being connected to said elongated support contacts.

15. The probe according to claim 14 wherein contacts on at least one of said portions are commutative so that said plug member contacts are electrically connected to said support member contacts irrespective of the rotative position of said plug member on said support.

16. The probe according to claim 13 further including a thermal insulating member provided on said support adjacent said probe.

17. The probe according to claim 13 further including a thermal insulating member comprising a refractory tube provided on said elongated support.

18. The probe according to claim 1 wherein said envelope is mounted on a support therefor, a cap member is mounted on said support, said cap member being shaped to enclose the otherwise exposed end of said envelope and said mass.

19. The probe according to claim 18 wherein said cap is fabricated from a material which melts or dissolves in said liquid metal.

\* \* \* \* \*